

# United States Patent [19]

Nire et al.

[11] 3,907,648

[45] Sept. 23, 1975

[54] **METHOD OF MANUFACTURING FORMED COKE FOR BLAST FURNACES WITHOUT CAUSING THE FUSION OF THE COKE**

[75] Inventors: Naomichi Nire, Takatsuki; Takeo Sakai, Nagareyama, both of Japan

[73] Assignees: Sumitomo Metal Industries Ltd.; Keihan Rentan Kogyo Co., Ltd., both of Japan

[22] Filed: Feb. 26, 1973

[21] Appl. No.: 335,868

## [30] Foreign Application Priority Data

Feb. 29, 1972 Japan..... 47-21240

[52] U.S. Cl..... 201/6; 44/10 R; 201/21; 201/23

[51] Int. Cl. C10B 45/02; C10L 5/00; C10B 53/00

[58] Field of Search..... 201/6, 5, 23, 22, 24, 21, 201/9; 75/42; 44/10 R, 23.1 R; 202/123, 130

## [56]

## References Cited

### UNITED STATES PATENTS

|           |         |                    |         |
|-----------|---------|--------------------|---------|
| 1,664,632 | 4/1928  | Koppers.....       | 202/130 |
| 2,200,371 | 5/1940  | Koppers.....       | 202/123 |
| 3,546,076 | 12/1970 | Muller et al. .... | 201/6   |
| 3,619,376 | 11/1971 | Patel et al. ....  | 201/6   |

Primary Examiner—Jack Sofer

Assistant Examiner—D. Sanders

Attorney, Agent, or Firm—Watson, Cole, Grindle & Watson

## [57]

## ABSTRACT

A method of manufacturing formed coke for blast furnaces enabling efficient and economical operation of the blast furnace, wherein the phenomenon of fusion of the formed coke is suppressed or substantially eliminated by appropriately adjusting the total dilatation of the coal material prior to briquetting and the Trommel strength of the coal briquette.

3 Claims, 7 Drawing Figures



**FIG.1**



**FIG.2**



**FIG.3A****FIG.3B****FIG.4A****FIG.4B****FIG.5**

**METHOD OF MANUFACTURING FORMED COKE FOR BLAST FURNACES WITHOUT CAUSING THE FUSION OF THE COKE**

This invention relates to improvements in the well known method of manufacturing formed coke. According to the method, formed coke is manufactured by carbonizing coal briquettes or cakes formed by pressure molding the blend coal which is composed of poor coking coal and non-coking coal as main materials and a small quantity of inert carbon material and coking coal as auxiliary materials and containing a proper amount of bituminous binder obtained from coal or petroleum.

This invention provides an improved method of manufacturing formed coke for blast furnaces without causing the fusion of the coke being carbonized, which is characterized in that the total dilatation of the blend material for the formed coke is made less than 27 percent, that the Trommel strength of the formed coke is made to be no less than 92 percent, and that the carbonization is done by using a coke oven where the carbonized formed coke can be discharged by its own weight.

Metallurgical coke, particularly blast furnace coke, is usually obtained by carbonizing a blended coal containing various hard coking coals in a conventional coke oven at a high temperature.

With the recent development of the steel industry, the material coal of good quality is getting increasingly difficult to obtain inexpensively and in large quantity. This trend will be further serious in the future.

To cope with this trend, the use of poor coking coal and non-coking coal, which occur in nature and are inexpensively available almost in any region of the world, as the main material in the manufacture of metallurgical coke have been investigated all over the world. Among various investigated method, the most effective and promising one is the formed coke method where mixture coal composed of poor coking coal and non-coking coal and containing a suitable quantity of binder such as pitch are molded with high pressure into briquettes or cakes having a constant form and then these coal briquettes are carbonized at a high temperature to obtain the formed coke. According to this method, particles of the coal having poor coking properties can be firmly bound together with the aid of binder and briquetting pressure, so that cokes having high strength can be obtained. Some excellent inventions relating to this method such as disclosed in Japanese Patent Publication No. 6678/1955, Japanese Patent Publication No. 8424/1965 and Japanese Patent Publication No. 5583/1971 are known. However, these inventions are not put to practice in industry from the grounds as will be given hereinafter.

According to the invention of the Japanese Patent Publication 6678/1955, formed coke is produced by adjusting the material proportions such that the caking component contained in the total material before briquetting is within a range between 60 and 66 percent. According to this method, however, good formed coke having a constant shape for blast furnaces cannot be obtained with material solely consisting of imported coal or containing 70 percent or more of imported coal since the fusion of the individual coal briquettes or cakes at the time of carbonization is severe. According to the invention of the Japanese Patent Publication No.

8424/1965, a step of charring treatment is involved, and it tends to increase the cost. Also, since low-temperature tar having small caking capacity is used as binder at the time of briquetting the char the strength of the formed coke is low. The method disclosed in the Japanese Patent Publication No. 5583/1971 requires 25 to 50 percent of coking coal to be incorporated into the coal material, so that, the material cost is high compared to the other methods. Also, it involves complicated steps of briquetting the material coal at a comparatively high temperature of 350° to 450°C and carbonizing the briquette by using sand at a high temperature of 900° to 1,200°C as the heat medium. Therefore, this method of production of formed coke on the industrial scale is impractical.

The present invention has been intended in view of the actual facts that coking coal of good quality is insufficient and that earlier inventions relating to the method of manufacturing formed coke using poor or non-coking coal as main material have not been put to practice in industry due to economical reasons. According to the invention there is provided a method of manufacturing high quality formed coke for blast furnaces economically and on the industrial scale by using poor coking coal and non-coking coal abundantly occurring in nature as main material. The inventors of the present invention noted that except for the economical aspect the prior-art for formed coke manufacturing techniques have not been put to practice in industry due to the following grounds;

1. If use is made of the conventional coke oven for producing formed coke, unlike the usual coke oven operation the formed coke after the carbonization cannot be discharged out of the oven by the pusher since the individual masses are not integrally fused.

2. Coke ovens other than the afore-mentioned conventional one, for example the continuous coke oven which is thoroughly suitable for the carbonization of formed coke, have been developed merely on the experimental scale or on a small pilot plant scale and are not industrially practicable.

3. According to the earlier researches and inventions conditions for blending material coals for producing high quality formed coke for blast furnaces and physical conditions of the formed coke are not fully satisfactory.

As the best prior-art coke oven for producing formed coke for blast furnaces, they studied such ovens as vertical coke oven and inclined coke oven, which do not require any pusher, and from which the carbonized product can be discharged by its own weight, and they have found that with these ovens it is possible to take the first step forward toward the industrialization. The vertical coke oven has a coke discharging door at the bottom of a coking chamber. After the carbonization, the coke is discharged by its own weight when the discharging door is opened. The inclined coke oven has an inclined coking chamber inclined at an angle greater than the angle of repose of the carbonized product, and the carbonized product can be discharged out of the oven by its own weight when a discharging door provided in a lower portion of the coking chamber is opened. While coke ovens of these types are well known to be used for producing coke from ordinal coking coal as the main material, their use for carbonization of formed coke for blast furnaces as according to this invention is unprecedented.

In the recent Japanese coal material situation, more than about 70 percent of coking coal for manufacturing blast furnace coke is imported, with less than 30 percent of domestic coking being used. The proportions of the imported coking coal is thought to be increased in the future. In the manufacture of formed coke for blast furnaces using imported coking coal as the main material, therefore, with the known techniques for instance the method of mixing materials according to Japanese Patent Publication No. 6678/1955, the fusion of the individual coal briquettes at the time of carbonization is severe, reducing the merits of the formed coke. It has been proved that it is necessary for the prevention of fusion of the formed coke to adjust the proportion of coal materials such that the total dilatation of the coal material after kneeding with addition of the binder such as pitch tar will not exceed 27 percent.

An object of the invention, accordingly, is to obviate drawbacks inherent in the prior-art techniques by the provision of a method of inexpensively manufacturing formed coke for blast furnaces by using a coking oven where the carbonized formed coke can be discharged by its own weight and without causing the fusion of the formed coke.

In the drawing.

FIG. 1 is a graph showing the relation between fusion ratio of the formed coke and total dilatation of the coal material according to the invention;

FIG. 2 is a graph showing the relation between fusion ratio of the formed coke and Trommel strength of the coal briquette;

FIG. 3A is a front view of a device for measuring the Trommel strength of the coal briquette used for the invention;

FIG. 3B is a side view of the device of FIG. 3A;

FIG. 4A is a front view of a vertical coke oven;

FIG. 4B is a side view of the oven of FIG. 4A; and

FIG. 5 is a side view of an inclined coke oven.

FIGS. 4 and 5 schematically show special coke ovens used for this invention.

Referring to FIG. 4, numeral 3 designates coking chamber, numeral 4 heating flue, numeral 5 charging hole, numeral 6 discharging door, and numeral 7 ascension pipe of coke oven gas. Referring to FIG. 5, which shows an inclined coke oven, numeral 8 designates coking chamber, numeral 9 charging hole, numeral 10 discharging door. The angle is greater than the angle of repose of the formed coke.

Referring now to FIG. 1, the total dilatation is a value determined by one of coal dilatation testing methods as specified in the German standard DIN-51739. If the material contains more than a certain quantity of strongly dilatable component, the coal briquette undergoes extraordinary dilatation during the carbonizing step, causing fusion of adjacent formed coke to one another, so that fused coke would result. To produce formed coke of a constant form with good yield, therefore, it is necessary to hold the dilatation of the mixture material below a predetermined level.

Further, in order to produce formed coke with high strength, for instance with JIS drum strength 15 mm index more than 92 percent, while preventing the fusion of coal briquettes being carbonized in the coke oven, it is necessary that the Trommel strength of the

coal briquette before carbonization is more than 92 percent in addition to the afore-mentioned total dilatation requirement. The Trommel strength is a value determined by a method similar to the method for measuring Trommel strength of steam locomotive engine fuel oval briquettes (JRS 61000-3593-09AR3) adopted by the Japanese National Railways. It is derived by loading 5 kg of a formed coke sample in a cylindrical iron container 2 having a length of 50 cm and a diameter of 50 cm and provided with three stirring plates each having a length of 50 cm, a width of 8 cm and a thickness of 0.32 cm, as shown in FIG. 3, rotating the container together with the sample at a speed of 25 rotations per minute for 2 minutes, then sifting the total sample with a square 15.9-mm-mesh sieve, dividing the weight of part of the sample on the sieve by the total sample weight, and multiplying the result by 100.

It will be seen that the Trommel strength represents the strength of bond between individual material coal particles constituting the coal briquette. If it is low, the bond of coal material particles is weak, so that coal briquette of low strength would be formed. The trommel strength of the coal briquette is proportional to the JIS drum strength 15-mm index of the formed coke. This relation will be apparent from FIG. 2.

If the Trommel strength of the coal briquette exceeds 92 percent, the fusion of the formed coke is extremely reduced, as will be seen from Tables 2 and 3.

As has been made apparent from the foregoing, the technical importance of the present invention resides in the following points:

1. A coke oven where the formed coke can be discharged by its own weight is used.

2. In the well-known method of manufacturing formed coke using poor coking coal and non-coking coal as main material, the total dilatation of the mixture material before briquetting is held below 27 percent, to thereby eliminate or avoid the fusion of the formed coke.

3. The requirement that the formed coke for blast furnaces should have a JIS drum strength 15-mm index more than 92 percent is met by having the Trommel strength of the coal briquette to be more than 92 percent. Doing so is also effective in suppressing the phenomenon of fusion of the formed coke.

Some embodiments of the invention will now be given.

## EMBODIMENT 1

Table 1 shows various kinds and qualities of coal used for research in the invention.

Coking coal and soft coking coal listed in Table 1 are used for producing blast furnace coke with a presently conventional coke oven.

The materials listed in Table 1 were used to prepare mixtures shown in Table 2. The mixtures were then kneaded in a kneader with steam blown into the kneader. Then, these mixtures are pressure molded into Masec type of 53 mm  $\times$  45 mm by using a briquette machine of double roll type with a roll diameter of 66 cm. The coal briquettes thus obtained were cooled down to a normal temperature and then sub-

Table 1

| Kind of coal            | Kind and Quality of Coal Used |                                    |                 |                                                    |                                                     |
|-------------------------|-------------------------------|------------------------------------|-----------------|----------------------------------------------------|-----------------------------------------------------|
|                         | Ash (%)<br>(Note 1)           | Volatile<br>matter (%)<br>(Note 1) | CBI<br>(Note 2) | Drum<br>strength<br>15-mm<br>index (%)<br>(note 3) | Informative<br>reference                            |
| Coking coal             | 9.4                           | 26.8                               | 6               | 93.1                                               |                                                     |
| Non-coking<br>coal      | 12.6                          | 32.2                               | Not coking      | 0                                                  |                                                     |
| Poor coking<br>coal (A) | 13.2                          | 20.7                               | 3               | 36.0                                               |                                                     |
| Poor coking<br>coal (B) | 8.1                           | 14.0                               | 1               | 0                                                  | Finely crushed<br>to a grain size<br>less than 3 mm |
| Petroleum coke          | 0.5                           | 10.9                               | Not coking      | 0                                                  |                                                     |
| Soft coking<br>coal     | 7.5                           | 42.8                               | 5               | 69.2                                               |                                                     |
| Hard pitch              | 0.2                           | 91.3                               | —               | —                                                  |                                                     |
| Coal tar                | 0.2                           | 91.3                               | —               | —                                                  |                                                     |

(Note 1) Determined by the method prescribed in JIS M 8812-1963 (Method for proximate analysis of coal and coke)

(Note 2) Determined by the method prescribed in JIS M 8801-1960 (Method for testing of coal)

(Note 3) Determined by the method prescribed in JIS K 2151-1960 (Method for testing of coke)

jected to high-temperature carbonization in a vertical coke oven as shown in FIG. 4 at a flue temperature of about 1250°C. After the carbonization the hot coke was discharged from the coke oven by opening the discharging door at the bottom of the oven and then water is sprinkled over the coke. Table 3 shows quality of coal briquette and formed coke obtained in this way.

As is shown in Table 3, the drum strength 15-mm index for the formed coke is above 92 percent in any of the tests. Thus, any sample can be used well for blast furnaces. In the test No. 1 the fusion factor of the formed coke is slightly high. The fusion factor here is calculated from an equation

30

$$\text{Fusion factor (in %)} = A/B \times 100$$

where A is the total weight of formed coke, and B is weight of coke with a grain size exceeding 50 mm. The 35 normal briquette not fused has average dimensions 48  $\times 48 \times 31$  mm.

The drum strength 15-mm index of the formed coke underwent fusion is 91.9 percent in the average, which is slightly lower than the formed coke strength required, but even the fused coke may be used for small-scale blast furnaces. In order to produce coke of a constant grain size with good yield, however, the fusion should be avoided as much as possible by appropriately adjusting the proportions of the coal materials used 45 coal briquette and the method of manufacturing coal briquette. Comparing the results in Table 3 and proportions of materials shown in Table 2, in the test No. 1, 5 percent of soft coking coal with a total dilatation of 24.1 percent is mixed. In the Test No. 2, the proportions of the coking coal and poor coking coal (A) are mixed 5 percent higher than those in the test No. 3. This difference in the material proportions is thought 50 to have delicate effects upon the phenomenon of fusion of the formed coke.

55

## EMBODIMENT 2

Table 4 shows results of testing for confirming the relation between the fusion factor of the formed coke mentioned in the previous embodiment 1 and the total dilatation of the all mixed materials prior to the briquetting and testing for seeking the relationship between Trommel strength of the coal briquette and quality of formed coke.

The method of producing coal briquette and formed coke is entirely the same as in the embodiment 1.

Table 2

| Test number          | Proportions of Coal Materials (in % by weight) |     |     |
|----------------------|------------------------------------------------|-----|-----|
|                      | 1                                              | 2   | 3   |
| Coking coal          | 10                                             | 15  | 10  |
| Non-coking coal      | 15                                             | 10  | 10  |
| Poor coking coal (A) |                                                | 15  | 10  |
| Poor coking coal (B) | 50                                             | 50  | 50  |
| Petroleum coke       | 10                                             | 10  | 10  |
| Soft coking coal     | 5                                              |     |     |
| Hard pitch           | 7                                              | 7   | 7   |
| Coal tar             | 3                                              | 3   | 3   |
| Total                | 100                                            | 100 | 100 |

Table 3

| Test number                                 | Quality of Coal Briquette and Formed Coke |       |       |       |
|---------------------------------------------|-------------------------------------------|-------|-------|-------|
|                                             | 1                                         | 2     | 3     |       |
| Material before<br>briquetting              | Ash (%)                                   | 7.4   | 7.5   | 7.8   |
|                                             | Volatile matter (%)                       | 24.1  | 21.3  | 23.6  |
|                                             | Total dilatation (%)                      | 39.0  | 28.7  | 27.5  |
| # Trommel strength of<br>coal briquette (%) |                                           | 93.0  | 94.1  | 92.6  |
| Formed<br>Coke                              | Ash (%)                                   | 9.4   | 9.3   | 9.8   |
|                                             | Volatile matter (%)                       | 1.0   | 0.9   | 0.9   |
|                                             | Drum strength<br>15-mm index (%)          | 92.55 | 92.40 | 93.75 |
|                                             | ASTM hardness factor                      | 62.0  | 60.5  | 66.6  |
|                                             | # Fusion ratio (%)                        | 16.6  | 10.1  | 2.0   |

Mark # indicates figures as an average for 10 measurements.

Table 4

| Results of Testing of Manufacture of Formed Coke |                                     | 4     | 5     | 6     | 7     |
|--------------------------------------------------|-------------------------------------|-------|-------|-------|-------|
| Test Number                                      |                                     |       |       |       |       |
| Proportions (in % by weight)                     | Coking coal                         | 10    | 10    | 10    | 13    |
|                                                  | Non-coking coal                     | 40    | 40    | 10    | 10    |
|                                                  | Poor coking coal (A)                | 15    | 10    | 10    | 10    |
|                                                  | Poor coking coal (B)                | 50    | 50    | 50    | 50    |
|                                                  | Petroleum coke                      | 5     | 10    | 10    | 10    |
|                                                  | Soft coking coal                    | 10    | 7     | 7     | 4     |
|                                                  | Pitch                               | 7     | 7     | 7     | 4     |
|                                                  | Coal tar                            | 3     | 3     | 3     | 3     |
|                                                  | Total                               | 100   | 100   | 100   | 100   |
| Coal material before briquetting                 | Ash (%)                             | 7.7   | 9.1   | 7.4   | 7.8   |
|                                                  | Volatile matter (%)                 | 24.9  | 22.8  | 22.7  | 22.5  |
|                                                  | # Total dilatation (%)              | 51.8  | 24.9  | 27.5  | 17.4  |
|                                                  | Trommel strength coal briquette (%) | 94.8  | 93.6  | 88.2  | 89.1  |
| Formed coke                                      | Ash (%)                             | 10.1  | 11.5  | 10.0  | 10.0  |
|                                                  | Volatile matter (%)                 | 1.2   | 1.1   | 1.1   | 1.0   |
|                                                  | Drum strength 15-mm index (%)       | 91.90 | 93.65 | 91.50 | 91.80 |
|                                                  | ASTM hardness factor                | 59.5  | 63.7  | 58.9  | 59.9  |
|                                                  | # Fusion factor (%)                 | 33.7  | 0.7   | 19.9  | 21.0  |

Mark # indicates figures as an average for 10 measurements.

In the test No. 4, the proportions are based on the method of adjusting the material proportions as set forth in the Japanese Patent Publication No. 6678/1950, that is, the material are set such that the caking component contained in the total material prior to briquetting is within a range between 60 and 66 percent. In this case, the fusion of the formed coke reaches as high as about 34 percent. This means that with the material mainly consisting of imported coal due to the recent coal situation, the method of the Japanese Patent Publication does not permit the manufacture of formed coke of a constant form with good yield.

In the test No. 5 the total dilatation of the mixture coal prior to briquetting is low, and the coal briquette has enough Trommel strength. Thus, in this example formed coke of high quality with very little fusion can be obtained.

In the test No. 6 the same material proportions as in the test No. 3 are used, and the briquetting is done with low pressure. In this case, Drum strength 15-mm index the formed coke is low, and the fusion factor is high.

In the test No. 7, the coal briquette is produced under the same conditions as in the embodiment 1 except for a reduction by 3 percent of the pitch in the binder and an increase by 3 percent of the coking coal. In this case, since the binder content is reduced, the Trommel strength of the coal briquette is reduced. As a result, the fusion of the formed coke reached 21 percent.

The results of the afore-mentioned embodiments 1 and 2 are shown in FIGS. 1 and 2.

It will be seen that by holding the total dilatation of the all material prior to the briquetting to be less than 27 percent and the Trommel strength of the coal briquette to be higher than 92 percent, it is possible to produce formed coke for blast furnaces having a constant form with very little fusion.

### EMBODIMENT 3

As has been mentioned earlier, the vertical coke oven used in this invention has a discharging door at the bottom of each coking chamber, and the coke after the end of carbonization can be discharged by its own

weight by opening the discharging door. Since no discharging operation by a pusher as is involved in the conventional coke oven is required, the vertical coke oven is best suited to the carbonization of formed coke. While it is known to use the coke oven of this type for the production of the conventional coke with material mainly composed of the coking coal, the use of this oven for the carbonization of formed coke for blast furnaces as according to this invention is unprecedented.

The inventors of this invention produced about 10,000 tons of formed coke for blast furnaces in about three months with the same material proportions and formed coal manufacturing conditions as in the test No. 3 mentioned above in the embodiment 1. Table 5 shows the quality of formed coke for blast furnaces obtained in this period and the quality of the ordinal coke for blast furnaces.

Table 5

| Kind of coke                  | Quality of Formed Coke for Blast Furnaces and Conventional Furnace Coke |                   |
|-------------------------------|-------------------------------------------------------------------------|-------------------|
|                               | Formed coke                                                             | Conventional coke |
| Total moisture (%)            | 2.2                                                                     | 3.4               |
| Ash (%)                       | 10.3                                                                    | 10.8              |
| Volatile matter (%)           | 0.9                                                                     | 0.9               |
| Total sulfur (%)              | 0.54                                                                    | 0.63              |
| Drum strength 15-mm index (%) | 93.3                                                                    | 92.2              |
| ASTM hardness factor          | 65.0                                                                    | 60.8              |
| Size distribution of coke     |                                                                         |                   |
| Above 100 mm (%)              | 0                                                                       | 0                 |
| 50 to 100 mm (%)              | 0.5                                                                     | 47.7              |
| 25 to 50 mm (%)               | 93.5                                                                    | 35.6              |
| 15 to 25 mm (%)               | 2.0                                                                     | 6.9               |
| Below 15 mm (%)               | 4.0                                                                     | 9.8               |
| Water absorption factor (%)   | 7.9                                                                     | 16.5              |

(Note 1) Figures for the conventional blast furnace coke indicate values after the cutting and screening.

(Note 2) The water absorption factor is the total moisture content (in percent by weight) obtained

after submerging coke with grain size of 30 to 40 mm in water for 24 hours.

The quality of the formed coke for blast furnaces according to the invention is superior to the coke produced with the conventional coke oven in the drum strength and grain size. Particularly, according to the invention, the grain size of the formed coke for blast furnaces is substantially within a range between 50 and 25 mm, and the proportion of powdery coke (-15 mm) is less than compared with the conventional coke. Also, the water absorption factor of the formed coke is about one half that of the conventional coke, which is very useful in the reduction of the coke ratio in the blast furnace.

It is to be emphasized that the formed coke for blast furnaces according to the invention, when used in the blast furnace, is superior to the cokes obtained according to earlier inventions and obtained with the conventional coke oven in the following points:

- a. It is economical since no expensive coking coal is used.
- b. Since its strength is high, the operation of the blast furnace can be stabilized and improved.
- c. Since the fusion is little, coke of uniform grain size can be obtained.
- d. Since the grain size is within a predetermined range, no coke cutter is required.
- e. Since the pulverization factor is low, the mass coke yield is high.

5

10

f. Since the grain size is uniform, the ventilation of the blast furnace can be improved.

g. Since the water absorption is low, the coke ratio of the blast furnace can be improved.

What is claimed is:

1. A method of manufacturing a blend of coal materials for use in producing formed coke for blast furnaces from a blend of different materials without causing the fusion of the coke, the blend being composed of 70 to 90 percent by weight of poor coking and non-coking coal as the main material, 20 to 0 percent by weight of auxiliary material including inert carbon substance and coking coal and 10 percent by weight of a binder so as to make the total of the blend material 100 percent, including blending various proportions of the different materials until both the average value of the total dilatation of the blend prior to briquetting is held to less than 27 percent and the Trrommel strength of the coal briquette is held to more than 92 percent.

2. A method of manufacturing formed coke for blast furnaces according to claim 1, wherein use is made of a coke oven permitting the discharging from the oven of the carbonized formed coke after carbonization of the coal briquette by the weight of the coke itself.

3. A method of manufacturing formed coke for blast furnaces according to claim 1, wherein the blend is produced into a coal briquette by pressure molding.

\* \* \* \* \*

25

30

35

40

45

50

55

60

65